



US010458013B2

(12) **United States Patent**  
**Fukuda et al.**

(10) **Patent No.:** **US 10,458,013 B2**  
(45) **Date of Patent:** **Oct. 29, 2019**

(54) **FERRITIC STAINLESS STEEL AND  
PROCESS FOR PRODUCING SAME**

(71) Applicant: **JFE STEEL CORPORATION**,  
Chiyoda-ku, Tokyo (JP)

(72) Inventors: **Kunio Fukuda**, Tokyo (JP); **Shin  
Ishikawa**, Tokyo (JP); **Mitsuyuki  
Fujisawa**, Tokyo (JP); **Katsuhisa  
Yamauchi**, Tokyo (JP); **Chikara Kami**,  
Tokyo (JP)

(73) Assignee: **JFE STEEL CORPORATION**,  
Chiyoda-ku, Tokyo (JP)

(\*) Notice: Subject to any disclaimer, the term of this  
patent is extended or adjusted under 35  
U.S.C. 154(b) by 37 days.

(21) Appl. No.: **15/538,335**

(22) PCT Filed: **Nov. 17, 2015**

(86) PCT No.: **PCT/JP2015/005728**

§ 371 (c)(1),  
(2) Date: **Jun. 21, 2017**

(87) PCT Pub. No.: **WO2016/103565**

PCT Pub. Date: **Jun. 30, 2016**

(65) **Prior Publication Data**

US 2017/0349995 A1 Dec. 7, 2017

(30) **Foreign Application Priority Data**

Dec. 24, 2014 (JP) ..... 2014-260776

(51) **Int. Cl.**  
**C23C 8/26** (2006.01)  
**C22C 38/42** (2006.01)

(Continued)

(52) **U.S. Cl.**  
CPC ..... **C23C 8/26** (2013.01); **C21D 1/06**  
(2013.01); **C21D 1/76** (2013.01); **C21D 9/46**  
(2013.01);

(Continued)

(58) **Field of Classification Search**

None  
See application file for complete search history.

(56) **References Cited**

U.S. PATENT DOCUMENTS

5,512,239 A 4/1996 Fujiwara et al.  
5,626,694 A 5/1997 Kawabata et al.  
(Continued)

FOREIGN PATENT DOCUMENTS

CN 102131946 A 7/2011  
CN 103643136 A 3/2014

(Continued)

OTHER PUBLICATIONS

Mar. 6, 2018, Notification of Reasons for Refusal issued by the  
Japan Patent Office in the corresponding Japanese Patent Application  
No. 2016-565875 with English language Concise Statement of  
Relevance.

(Continued)

*Primary Examiner* — Keith Walker

*Assistant Examiner* — Adil A. Siddiqui

(74) *Attorney, Agent, or Firm* — Kenja IP Law PC

(57) **ABSTRACT**

Provided is a ferritic stainless steel having a chemical  
composition containing, in mass %: 0.003% to 0.025% of C;  
0.05% to 1.00% of Si; 0.05% to 1.00% of Mn; 0.04% or less  
of P; 0.01% or less of S; 16.0% to 23.0% of Cr; 0.20% to  
0.80% of Cu; 0.05% to 0.60% of Ni; 0.20% to 0.70% of Nb;  
0.005% to 0.020% of N; and the balance being Fe and  
incidental impurities, in which a nitrogen-enriched layer is  
present that has a nitrogen concentration peak value of 0.03

(Continued)



mass % to 0.30 mass % at a depth of within 0.05  $\mu\text{m}$  of a surface of the steel.

**4 Claims, 2 Drawing Sheets**

**(51) Int. Cl.**

*C22C 38/02* (2006.01)  
*C21D 1/76* (2006.01)  
*C22C 38/00* (2006.01)  
*C21D 9/46* (2006.01)  
*C22C 38/48* (2006.01)  
*C22C 38/04* (2006.01)  
*C21D 1/06* (2006.01)  
*C22C 38/54* (2006.01)  
*C22C 38/06* (2006.01)  
*C22C 38/44* (2006.01)  
*C22C 38/46* (2006.01)  
*C22C 38/50* (2006.01)

**(52) U.S. Cl.**

CPC ..... *C22C 38/00* (2013.01); *C22C 38/001* (2013.01); *C22C 38/02* (2013.01); *C22C 38/04* (2013.01); *C22C 38/06* (2013.01); *C22C 38/42* (2013.01); *C22C 38/44* (2013.01); *C22C 38/46* (2013.01); *C22C 38/48* (2013.01); *C22C 38/50* (2013.01); *C22C 38/54* (2013.01)

**(56)**

**References Cited**

U.S. PATENT DOCUMENTS

|                   |         |                          |
|-------------------|---------|--------------------------|
| 8,383,034 B2      | 2/2013  | Fukuda et al.            |
| 9,611,525 B2      | 4/2017  | Hiraide et al.           |
| 2008/0057357 A1 * | 3/2008  | Uchiyama ..... C23C 8/26 |
|                   |         | 429/467                  |
| 2010/0061878 A1   | 3/2010  | Fukuda et al.            |
| 2010/0272594 A1   | 10/2010 | Hiraide                  |
| 2011/0176953 A1   | 7/2011  | Hiraide et al.           |
| 2012/0085513 A1   | 4/2012  | Oku et al.               |
| 2014/0069619 A1   | 3/2014  | Hiraide et al.           |
| 2015/0376732 A1 * | 12/2015 | Hamada ..... C21D 9/46   |
|                   |         | 148/610                  |
| 2017/0321310 A1 * | 11/2017 | Hatano ..... C21D 1/76   |

FOREIGN PATENT DOCUMENTS

|    |                 |         |
|----|-----------------|---------|
| JP | S5861220 A      | 4/1983  |
| JP | S6013060 A      | 1/1985  |
| JP | H01168811 A     | 7/1989  |
| JP | H01176094 A     | 7/1989  |
| JP | H107216447 A    | 8/1995  |
| JP | H07292446 A     | 11/1995 |
| JP | H08109443 A     | 4/1996  |
| JP | H10176249 A     | 6/1998  |
| JP | H11236654 *     | 8/1999  |
| JP | 2000212704 A    | 8/2000  |
| JP | 2001032051 A    | 2/2001  |
| JP | 2008001945 A    | 1/2008  |
| JP | 2008190035 A    | 8/2008  |
| JP | 2009174040 A    | 8/2009  |
| JP | 2009197293 A    | 9/2009  |
| JP | 2009228036 A    | 10/2009 |
| JP | 2010121208 A    | 6/2010  |
| JP | 2010285683 A    | 12/2010 |
| JP | 2013014796 A    | 1/2013  |
| KR | 1020130125823 A | 11/2013 |
| WO | 2010047131 A1   | 4/2010  |
| WO | 2015141145 A1   | 9/2015  |

OTHER PUBLICATIONS

Feb. 24, 2018, Office Action issued by the State Intellectual Property Office in the corresponding Chinese Patent Application No. 201580070725.0 with English language Search Report.

Jan. 2, 2018, Extended European Search Report issued by the European Patent Office in the corresponding European Patent Application No. 15872143.1.

Aug. 9, 2018, Office Action issued by the Korean Intellectual Property Office in the corresponding Korean Patent Application No. 10-2017-7017965 with English language concise statement of relevance.

Feb. 23, 2016, International Search Report issued in the International Patent Application No. PCT/JP2015/005728.

Jul. 4, 2016, Office Action issued by Taiwan Intellectual Property Office in the corresponding Taiwanese Patent Application No. 104142961 with English language concise statement of relevance.

Jan. 3, 2019, Office Action issued by the State Intellectual Property Office in the corresponding Chinese Patent Application No. 201580070725.0 with English language search report.

\* cited by examiner

FIG. 1



*FIG. 2A**FIG. 2B*

## FERRITIC STAINLESS STEEL AND PROCESS FOR PRODUCING SAME

### TECHNICAL FIELD

The present disclosure relates to a ferritic stainless steel having excellent corrosion resistance and displaying good brazing properties when brazing is carried out at high temperature using a Ni-containing brazing metal, and to a process for producing the ferritic stainless steel.

### BACKGROUND

In recent years, there has been demand for further improvement of automobile fuel efficiency and exhaust gas purification from a standpoint of environmental protection. Consequently, adoption of exhaust heat recovery units and EGR (Exhaust Gas Recirculation) coolers in automobiles continues to increase.

An exhaust heat recovery unit is an apparatus that improves fuel efficiency by, for example, using heat from engine coolant for automobile heating and using heat from exhaust gas to warm up engine coolant in order to shorten warming-up time when the engine is started up. The exhaust heat recovery unit is normally located between a catalytic converter and a muffler, and includes a heat exchanger part formed by a combination of pipes, plates, fins, side plates, and so forth, and entry and exit pipe parts. Usually, fins, plates, and the like have a small sheet thickness (about 0.1 mm to 0.5 mm) to reduce back pressure resistance, and side plates, pipes, and the like have a large sheet thickness (about 0.8 mm to 1.5 mm) to ensure strength. Exhaust gas enters the heat exchanger part through the entry pipe, transfers its heat to a coolant via a heat-transfer surface such as a fin, and is discharged from the exit pipe. Bonding and assembly of plates, fins, and so forth forming the heat exchanger part of an exhaust heat recovery unit such as explained above is mainly carried out by brazing using a Ni-containing brazing metal.

An EGR cooler includes a pipe for intake of exhaust gas from an exhaust manifold or the like, a pipe for returning the exhaust gas to a gas intake-side of an engine, and a heat exchanger for cooling the exhaust gas. The EGR cooler more specifically has a structure in which a heat exchanger including both a water flow passage and an exhaust gas flow passage is located on a path along which exhaust gas is returned to the gas intake-side of the engine from the exhaust manifold. Through the structure described above, high-temperature exhaust gas at the exhaust-side is cooled by the heat exchanger and the cooled exhaust gas is returned to the gas intake-side such as to lower the combustion temperature of the engine. Accordingly, this structure forms a system for inhibiting  $\text{NO}_x$  production, which tends to occur at high temperatures. The heat exchanger part of the EGR cooler is made by overlapping thin fins and plates, for reductions in weight, size, cost, etc. Bonding and assembly of these thin plates is mainly carried out by brazing using a Ni-containing brazing metal.

Since bonding and assembly for a heat exchanger part in an exhaust heat recovery unit or an EGR cooler such as described above are carried out by brazing using a Ni-containing brazing metal, materials used in the heat exchanger part are expected to have good brazing properties with respect to the Ni-containing brazing metal. Moreover, a heat exchanger part such as described above is expected to be highly resistant to oxidation caused by high-temperature exhaust gas passing through the heat exchanger part. The

exhaust gas includes small amounts of nitrogen oxides ( $\text{NO}_x$ ), sulfur oxides ( $\text{SO}_x$ ), and hydrocarbons (HC) that may condense in the heat exchanger to form a strongly acidic and corrosive condensate. Therefore, materials used in a heat exchanger part such as described above are expected to have corrosion resistance at normal temperatures. In particular, because brazing heat treatment is carried out at high temperature, it is necessary to prevent formation of a Cr depletion layer due to preferential reaction of Cr at grain boundaries with C and N, which is referred to as sensitization, in order to ensure that corrosion resistance is obtained.

For the reason described above, heat exchanger parts of exhaust heat recovery units and EGR coolers are normally made using an austenitic stainless steel such as SUS316L or SUS304L that has a reduced carbon content and is resistant to sensitization. However, austenitic stainless steels suffer from problems such as high cost due to having high Ni content, and also poor fatigue properties and poor thermal fatigue properties at high temperatures due to its large thermal expansion when used in an environment in which constraining force is received at high temperature and with severe vibration, such as when used as a component located peripherally to an exhaust manifold.

Therefore, steels other than austenitic stainless steels are being considered for use in heat exchanger parts of exhaust heat recovery units and EGR coolers.

For example, PTL 1 discloses, as a heat exchanger component of an exhaust heat recovery unit, a ferritic stainless steel in which Mo, Ti, or Nb are added and Si and Al content is reduced. PTL 1 discloses that addition of Ti or Nb prevents sensitization by stabilizing C and N in the steel as carbonitrides of Ti and Nb and that reduction of Si and Al content improves brazing properties.

PTL 2 discloses, as a component for a heat exchanger of an exhaust heat recovery unit, a ferritic stainless steel having excellent condensate corrosion resistance in which Mo content is defined by Cr content, and Ti and Nb content is defined by C and N content.

Furthermore, PTL 3 discloses, as a material for an EGR cooler, a ferritic stainless steel in which added amounts of components such as Cr, Cu, Al, and Ti satisfy a certain relationship.

Additionally, PTL 4 and 5 disclose, as a component of an EGR cooler and a material for a heat exchanger part of an EGR cooler, a ferritic stainless steel containing 0.3 mass % to 0.8 mass % of Nb and a ferritic stainless steel containing 0.2 mass % to 0.8 mass % of Nb.

### CITATION LIST

#### Patent Literature

- PTL 1: JP H7-292446 A
- PTL 2: JP 2009-228036 A
- PTL 3: JP 2010-121208 A
- PTL 4: JP 2009-174040 A
- PTL 5: JP 2010-285683 A

### SUMMARY

#### Technical Problem

However, the steel disclosed in each of PTL 1 and PTL 2 has a problem of being expensive as Mo, which is a high cost raw material, needs to be contained. Besides, in the case where a Ni-containing brazing metal (e.g. BNi-2, BNi-5, or the like in JIS (JIS Z 3265)) having a high brazing tempera-

ture is used for such steel, a brazing failure may occur or sufficient brazing property may not be achieved.

PTL 3, PTL 4, and PTL 5 each disclose steel containing Cu which is cheaper than Mo. With Cu-containing steel, however, sufficient brazing property is not always achieved as seen, for example, in the case where the brazing metal does not sufficiently penetrate into the crevice between the overlapped steel sheets when overlapping and brazing the steel sheets or satisfactory bond strength is not attained. This seems to be because, with Cu-containing steel, a Cr oxide layer which decreases brazing property tends to form when performing high-temperature brazing using a Ni-containing brazing metal.

Moreover, PTL 4 and PTL 5 each disclose steel containing neither Mo nor Cu. Such steel, however, lacks corrosion resistance after brazing.

It could be helpful to provide ferritic stainless steel that, without containing a large amount of an expensive element such as Mo, has favorable brazing property when performing high-temperature brazing using a Ni-containing brazing metal and also has excellent corrosion resistance, and a process for producing the same.

#### Solution to Problem

Assuming that Cu is contained from the viewpoint of saving production cost and ensuring corrosion resistance, we conducted diligent investigation in which we produced Cu-containing ferritic stainless steel using various different chemical compositions and production conditions, and investigated various properties thereof, particularly brazing properties when brazing is carried out at high temperature using a Ni-containing brazing metal.

As a result of this investigation, we discovered that it is possible to prevent formation of an oxide film of Cr during brazing by optimizing the chemical composition and subjecting the steel to heat treatment in a controlled atmosphere prior to brazing such that a specific nitrogen-enriched layer is formed in a surface layer part of the steel. It was also discovered that through formation of this nitrogen-enriched layer, good brazing properties can be satisfactorily obtained even when brazing is carried out at high temperature using a Ni-containing brazing metal.

Based on these findings, we conducted further investigation which eventually led to the present disclosure.

Specifically, the primary features of the present disclosure are as follows.

1. A ferritic stainless steel comprising a chemical composition containing (consisting of), in mass %:
  - 0.003% to 0.025% of C;
  - 0.05% to 1.00% of Si;
  - 0.05% to 1.00% of Mn;
  - 0.04% or less of P;
  - 0.01% or less of S;
  - 16.00% to 23.00% of Cr;
  - 0.20% to 0.80% of Cu;
  - 0.05% to 0.60% of Ni;
  - 0.20% to 0.70% of Nb;
  - 0.005% to 0.020% of N; and
  - the balance being Fe and incidental impurities, wherein a nitrogen-enriched layer is present that has a nitrogen concentration peak value of 0.03 mass % to 0.30 mass % at a depth of within 0.05  $\mu\text{m}$  of a surface of the steel.
2. The ferritic stainless steel described above in 1, wherein the chemical composition further contains, in mass %, one or more of:

0.05% to 0.20% of Mo;

0.01% to 0.15% of Al;

0.01% to 0.15% of Ti;

0.01% to 0.20% of V;

5 0.0003% to 0.0030% of Ca; and

0.0003% to 0.0030% of B.

3. A process for producing the ferritic stainless steel described above in 1 or 2, the process including:

10 hot rolling a slab having the chemical composition described above in 1 or 2 to form a hot-rolled sheet;

optionally performing hot-rolled sheet annealing on the hot-rolled sheet; and

15 performing a combination of cold rolling and annealing on the hot-rolled sheet one or more times,

15 wherein a cold-rolled sheet after subjection to final cold rolling is heated in final annealing with a dew point of an atmosphere in a temperature range of 600° C. to 800° C. being -20° C. or lower, and subjected to a nitrogen-enriched layer forming treatment at a temperature of 900° C. or higher in an atmosphere of -20° C. or lower in dew point and 5 vol % or more in nitrogen concentration.

#### Advantageous Effect

25 According to the present disclosure, a ferritic stainless steel can be obtained that has excellent corrosion resistance and that displays good brazing properties when brazing is carried out at high temperature using a Ni-containing brazing metal.

#### BRIEF DESCRIPTION OF THE DRAWINGS

In the accompanying drawings:

FIG. 1 is a schematic view illustrating a test material used to evaluated joint gap infiltration by a brazing metal; and

35 FIG. 2 schematically illustrates a tensile test piece used to evaluate joint strength of a brazed part, wherein FIG. 2A illustrates one side of the tensile test piece prior to brazing and FIG. 2B illustrates the entire tensile test piece after 40 brazing.

#### DETAILED DESCRIPTION

The following provides a specific description of the 45 present disclosure.

First, the reasons for limiting the chemical composition of the steel to the aforementioned range in the present disclosure are explained. Hereinafter, the unit “%” relating to the content of elements in the chemical composition of the steel 50 refers to “mass %” unless specified otherwise.

C: 0.003% to 0.025%

Strength of the steel increases with increasing C content whereas workability of the steel increases with decreasing C content. Herein, the C content is required to be 0.003% or

55 greater in order to obtain sufficient strength. However, if the C content is greater than 0.025%, workability noticeably decreases and sensitization tends to occur more easily due to Cr carbide precipitation at grain boundaries, promoting a decrease in corrosion resistance. Accordingly, the C content 60 is in a range of 0.003% to 0.025%. The C content is preferably 0.005% or more. The C content is preferably 0.020% or less. The C content is more preferably 0.005% or more. The C content is more preferably 0.015% or less.

Si: 0.05% to 1.00%

Si is a useful element as a deoxidizer. This effect is obtained through Si content of 0.05% or greater. However, if Si content is greater than 1.00%, workability noticeably

decreases and forming becomes difficult. Accordingly, the Si content is in a range of 0.05% to 1.00%. The Si content is preferably 0.10% or more. The Si content is preferably 0.50% or less.

Mn: 0.05% to 1.00%

Mn has a deoxidizing effect that is obtained through Mn content of 0.05% or greater. However, excessive Mn addition leads to loss of workability due to solid solution strengthening. Furthermore, excessive Mn decreases corrosion resistance by promoting precipitation of MnS, which acts as a starting point for corrosion. Therefore, Mn content of 1.00% or less is appropriate. Accordingly, the Mn content is in a range of 0.05% to 1.00%. The Mn content is preferably 0.15% or more. The Mn content is preferably 0.35% or less.

P: 0.04% or Less

P is an element that is incidentally included in the steel. However, excessive P content reduces weldability and facilitates intergranular corrosion. This trend is noticeable if the P content is greater than 0.04%. Accordingly, the P content is 0.04% or less. The P content is preferably 0.03% or less.

However, since excessive dephosphorization leads to increased refining time and costs, the P content is preferably 0.005% or greater.

S: 0.01% or Less

S is an element that is incidentally contained in the steel, and that promotes MnS precipitation and decreases corrosion resistance if S content is greater than 0.01%. Accordingly, the S content is 0.01% or less. The S content is preferably 0.007% or less. Meanwhile, excessive desulfurization incurs longer refining time and higher cost, and so the S content is preferably 0.0005% or more.

Cr: 16.0% to 23.0%

Cr is an important element for ensuring corrosion resistance of the stainless steel. Adequate corrosion resistance after brazing is not obtained if Cr content is less than 16.0%. However, excessively adding Cr causes the formation of a Cr oxide layer when performing high-temperature brazing using a Ni-containing brazing metal, which degrades brazing properties. Accordingly, the Cr content is in a range of 16.0% to 23.0%. The Cr content is preferably 18.0% or more. The Cr content is preferably 21.5% or less.

Cu: 0.20% to 0.80%

Cu is an element that enhances corrosion resistance. This effect is obtained through Cu content of 0.20% or greater. However, Cu content of greater than 0.80% reduces hot workability. Accordingly, the Cu content is in a range of 0.20% to 0.80%. The Cu content is preferably 0.22% or more. The Cu content is preferably 0.60% or less. The Cu content is more preferably 0.30% or more. The Cu content is more preferably 0.50% or less.

Ni: 0.05% to 0.60%

Ni is an element that effectively contributes to improving toughness and to improving crevice corrosion resistance when contained in an amount of 0.05% or greater. However, Ni content of greater than 0.60% increases stress corrosion crack sensitivity. Furthermore, Ni is an expensive element that leads to increased costs. Accordingly, the Ni content is in a range of 0.05% to 0.60%. The Ni content is preferably 0.10% or more. The Ni content is preferably 0.50% or less.

Nb: 0.20% to 0.70%

Nb is an element that combines with C and N and suppresses degradation of corrosion resistance (sensitization) due to the precipitation of Cr carbonitride, in the same way as Ti described later. Nb also has an effect of forming the nitrogen-enriched layer by combining with nitrogen. These effects are obtained through Nb content of 0.20% or

greater. However, if the Nb content exceeds 0.70%, weld cracking occurs easily in the weld. Accordingly, the Nb content is in a range of 0.20% to 0.70%. The Nb content is preferably 0.25% or more. The Nb content is preferably 0.60% or less. The Nb content is more preferably 0.30% or more. The Nb content is preferably 0.50% or less.

N: 0.005% to 0.020%

N is an important element for preventing formation of Al or Ti oxide film during brazing and improving brazing properties due to formation of the nitrogen-enriched layer. N content is required to be 0.005% or greater in order to form the nitrogen-enriched layer. However, N content of greater than 0.020% facilitates sensitization and reduces workability. Accordingly, the N content is in a range of 0.005% to 0.020%. The N content is preferably 0.007% or more. The N content is preferably 0.015% or less. The N content is more preferably 0.007% or more. The N content is more preferably 0.010% or less.

In addition to the basic components described above, the chemical composition in the present disclosure may appropriately further contain the following elements as required.

Mo: 0.05% to 0.20%

Mo improves corrosion resistance by stabilizing a passivation film of the stainless steel. This effect is obtained through Mo content of 0.05% or greater. Since Mo is an expensive element, the Mo content is preferably 0.20% or less. Accordingly, in a situation in which Mo is contained in the steel, the Mo content is in a range of 0.05% to 0.20%.

Al: 0.01% to 0.15%

Al is an element useful for deoxidation. This effect is achieved when the Al content is 0.01% or more. If an Al oxide film forms on the surface of steel during brazing, however, the spreading property and adhesion of the brazing metal decrease, making brazing difficult. Al oxide film formation during brazing is prevented in the present disclosure through formation of the nitrogen-enriched layer in the surface layer of the steel, but it is not possible to adequately prevent formation of Al oxide film if Al content is greater than 0.15%. Accordingly, in a situation in which Al is contained in the steel, the Al content is in a range of 0.01% to 0.15%. The Al content is preferably 0.05% or more. The Al content is preferably 0.10% or less.

Ti: 0.01% to 0.15%

Ti is an element that prevents the precipitation of Cr carbonitride, which decreases corrosion resistance (sensitization), since Ti combines with C and N preferentially. This effect is obtained through Ti content of 0.01% or greater. However, Ti is not a preferable element from a viewpoint of brazing properties. The reason for this is that Ti is an active element with respect to oxygen and thus brazing properties are decreased as a result of a Ti oxide film being formed during brazing. Formation of Ti oxide film during brazing is prevented in the present disclosure through formation of a nitrogen-enriched layer in a surface layer of the steel, but brazing properties tend to be decreased if Ti content is greater than 0.15%. Accordingly, in a situation in which Ti is contained in the steel, the Ti content is in a range of 0.01% to 0.15%. The Ti content is preferably 0.05% or more. The Ti content is preferably 0.10% or less.

V: 0.01% to 0.20%

V combines with C and N contained in the steel and prevents sensitization in the same way as Ti. V also has an effect of forming the nitrogen-enriched layer by combining with nitrogen. These effects are obtained through V content of 0.01% or greater. On the other hand, V content of greater than 0.20% reduces workability. Accordingly, in a situation in which V is contained in the steel, the V content is in a

range of 0.01% to 0.20%. The V content is preferably 0.01% or more. The V content is preferably 0.15% or less. The V content is more preferably 0.01% or more. The V content is more preferably 0.10% or less.

Ca: 0.0003% to 0.0030%

Ca improves weldability by improving penetration of a welded part. This effect is obtained through Ca content of 0.0003% or greater. However, Ca content of greater than 0.0030% decreases corrosion resistance by combining with S to form CaS. Accordingly, in a situation in which Ca is contained in the steel, the Ca content is in a range of 0.0003% to 0.0030%. The Ca content is preferably 0.0005% or more. The Ca content is preferably 0.0020% or less.

B: 0.0003% to 0.0030%

B is an element that improves resistance to secondary working brittleness. This effect is exhibited when B content is 0.0003% or greater. However, B content of greater than 0.0030% reduces ductility due to solid solution strengthening. Accordingly, in a situation in which B is contained in the steel, the B content is in a range of 0.0003% to 0.0030%.

Through the above description, the chemical composition of the presently disclosed ferritic stainless steel has been explained.

In the chemical composition according to the present disclosure, components other than those listed above are Fe and incidental impurities.

In the presently disclosed ferritic stainless steel, it is very important that the chemical composition of the steel is appropriately controlled such as to be in the range described above and that a nitrogen-enriched layer such as described below is created in the surface layer part of the steel by performing heat treatment in a controlled atmosphere prior to brazing.

Nitrogen concentration peak value at depth of within 0.05  $\mu\text{m}$  of surface: 0.03 mass % to 0.30 mass %

In the presently disclosed ferritic stainless steel, a nitrogen-enriched layer is formed that has a nitrogen concentration peak value of 0.03 mass % to 0.30 mass % at a depth of within 0.05  $\mu\text{m}$  of the surface of the steel. This nitrogen-enriched layer can suppress formation of an oxide film of Cr or the like at the steel surface during brazing and, as a result, can improve brazing properties when a Ni-containing brazing metal is used.

N in the nitrogen-enriched layer described above combines with Cr, Nb, Ti, Al, V, and the like in the steel. The following describes a mechanism which we consider to be responsible for the nitrogen-enriched layer suppressing formation of an oxide film of Cr or the like during brazing.

Specifically, formation of the nitrogen-enriched layer causes Cr or the like present in the surface layer part of the steel to combine with N, so that the Ti and Al cannot diffuse to the surface of the steel. Furthermore, Cr or the like present inward of the nitrogen-enriched layer cannot diffuse to the surface of the steel because the nitrogen-enriched layer acts as a barrier. Accordingly, formation of an oxide film of Cr or the like is suppressed as a result of Cr or the like in the steel not diffusing to the surface.

Herein, formation of an oxide film of Cr or the like at the steel surface cannot be adequately prevented during brazing if the nitrogen concentration peak value is less than 0.03 mass %. On the other hand, the surface layer part hardens if the nitrogen concentration peak value is greater than 0.30 mass %, making defects more likely to occur, such as fin plate cracking due to hot cycles of an engine or the like.

Therefore, the nitrogen concentration peak value at a depth of within 0.05  $\mu\text{m}$  of the surface has a value in a range of 0.03 mass % to 0.30 mass %. The nitrogen concentration

peak value is preferably 0.05 mass % or more. The nitrogen concentration peak value is preferably 0.20 mass % or less.

Note that the nitrogen concentration peak value at a depth of within 0.05  $\mu\text{m}$  of the surface referred to herein can for example be calculated by measuring nitrogen concentration in the steel in a depth direction by glow discharge optical emission spectroscopy, dividing a maximum value for nitrogen concentration at a depth of within 0.05  $\mu\text{m}$  of the steel surface by a measured value for nitrogen concentration at a depth of 0.50  $\mu\text{m}$ , and multiplying the resultant value by the nitrogen concentration of the steel obtained through chemical analysis.

Furthermore, the nitrogen-enriched layer described herein refers to a region in which nitrogen is enriched due to permeation of nitrogen from the surface of the steel. The nitrogen-enriched layer is formed in the surface layer part of the steel and more specifically in a region spanning for a depth of approximately 0.005  $\mu\text{m}$  to 0.05  $\mu\text{m}$  in the depth direction from the surface of the steel.

15 The following describes a suitable production process for the presently disclosed ferritic stainless steel.

16 Molten steel having the chemical composition described above is prepared by steelmaking through a commonly known process such as using a converter, an electric heating furnace, or a vacuum melting furnace, and is subjected to continuous casting or ingot casting and blooming to obtain a steel raw material (slab).

17 The steel raw material is hot rolled to obtain a hot-rolled sheet either directly without prior heating or after heating at 1100° C. to 1250° C. for 1 hour to 24 hours. The hot-rolled sheet is normally subjected to hot-rolled sheet annealing at 900° C. to 1100° C. for 1 minute to 10 minutes, but depending on the intended use, this hot-rolled sheet annealing may be omitted.

18 Thereafter, the hot-rolled sheet is subjected to a combination of cold rolling and annealing to obtain a product steel sheet.

19 The cold rolling is preferably performed with a rolling reduction rate of 50% or greater in order to improve shape adjustment, ductility, bendability, and press formability. Furthermore, the cold rolling and annealing process may be repeated two or more times.

20 Herein, it is necessary to form the above-described nitrogen-enriched layer in order to obtain the presently disclosed ferritic stainless steel. Treatment for forming the nitrogen-enriched layer is preferably performed (on the sheet after subjection to the cold rolling during final annealing (finish annealing) carried out after the cold rolling).

21 Note that treatment for forming the nitrogen-enriched layer can be performed in a separate step to annealing, such as, for example, after a component has been cut from the steel sheet. However, it is advantageous in terms of production efficiency to form the nitrogen-enriched layer during the final annealing (finish annealing) carried out after the cold rolling because this allows the nitrogen-enriched layer to be formed without increasing the number of production steps.

22 The following describes conditions in treatment for forming the nitrogen-enriched layer.

Dew Point: -20° C. or Lower

23 If the dew point is higher than -20° C., a nitrogen-enriched layer is not formed because nitrogen from the surrounding atmosphere does not permeate into the steel due to formation of an oxide film at the surface of the steel. Accordingly, the dew point is -20° C. or lower. The dew point is preferably -30° C. or lower, and more preferably -40° C. or lower. The lower limit is not particularly limited, but is typically about -55° C.

Treatment Atmosphere Nitrogen Concentration: 5 Vol % or Greater

If the nitrogen concentration of the treatment atmosphere is less than 5 vol %, a nitrogen-enriched layer is not formed because an insufficient amount of nitrogen permeates into the steel. Accordingly, the nitrogen concentration of the treatment atmosphere is 5 vol % or greater. The nitrogen concentration of the treatment atmosphere is preferably 10 vol % or greater. The remainder of the treatment atmosphere, besides nitrogen, is preferably one or more selected from hydrogen, helium, argon, neon, CO, and CO<sub>2</sub>. The nitrogen concentration of the treatment atmosphere may be 100 vol %.

Treatment Temperature: 900° C. or Higher

If the treatment temperature is lower than 900° C., a nitrogen-enriched layer is not formed because nitrogen in the treatment atmosphere does not permeate into the steel. Accordingly, the treatment temperature is 900° C. or higher. The treatment temperature is preferably 950° C. or higher. However, the treatment temperature is preferably 1100° C. or lower because a treatment temperature of higher than 1100° C. leads to deformation of the steel. The treatment temperature is more preferably 1050° C. or lower.

The treatment time is preferably in the range of 5 seconds to 3600 seconds. The reason for this is that nitrogen in the treatment atmosphere does not sufficiently permeate into the steel if the treatment time is shorter than 5 seconds, whereas the effects of treatment reach saturation if the treatment time is longer than 3600 seconds. The treatment time is preferably 30 seconds or more. The treatment time is preferably 300 seconds or less.

Although the conditions of the nitrogen-enriched layer forming treatment have been described above, it is important to appropriately control not only the conditions of the nitrogen-enriched layer forming treatment but also the heating condition in the final annealing (i.e. the heating condition before the nitrogen-enriched layer creation treatment), in order to form a desired nitrogen-enriched layer.

Dew point of atmosphere in temperature range of 600° C. to 800° C. during heating in final annealing: -20° C. or lower

If the dew point of the atmosphere in the temperature range of 600° C. to 800° C. during heating in the final annealing is high, an oxide forms on the surface of steel. Such an oxide prevents the permeation of nitrogen in the atmosphere into the steel during the aforementioned nitrogen-enriched layer forming treatment. If such an oxide exists on the surface of steel, the nitriding of the surface layer of the steel does not progress even when the conditions of the nitrogen-enriched layer forming treatment are appropriately controlled, making it difficult to form a desired nitrogen-enriched layer. The dew point of the atmosphere in the temperature range of 600° C. to 800° C. during heating in the final annealing is therefore -20° C. or lower, and preferably -35° C. or lower. The lower limit is not particularly limited, but is typically about -55° C.

Although descaling may be performed after final annealing (finish annealing) by normal pickling or polishing, from a viewpoint of production efficiency, it is preferable to perform descaling by adopting the high-speed pickling process in which mechanical grinding is performed using a brush roller, a polishing powder, shot blasting, or the like, and pickling is subsequently performed in a nitrohydrochloric acid solution.

In a situation in which treatment for forming the nitrogen-enriched layer is performed during final annealing (finish annealing), care should be taken to adjust the amount of

pickling or polishing in order that the nitrogen-enriched layer that has been formed is not removed.

## EXAMPLES

Steels having the chemical compositions shown in Table 1 were each prepared by steelmaking using a 50 kg small vacuum melting furnace. Each resultant steel ingot was heated to 1150° C. in a furnace purged with Ar gas and was subsequently subjected to hot-rolling to obtain a hot-rolled sheet having a thickness of 3.5 mm. Next, each of the hot-rolled sheets was subjected to hot-rolled sheet annealing at 1030° C. for 1 minute and shot blasting of the surface thereof with glass beads was performed. Thereafter, descaling was performed by carrying out pickling in which the sheet was immersed in a 200 g/l sulfuric acid solution at a temperature of 80° C. for 120 seconds and was subsequently immersed in a mixed acid of 150 g/l of nitric acid and 30 g/l of hydrofluoric acid at a temperature of 55° C. for 60 seconds.

Next, each hot-rolled and annealed sheet was subjected to cold-rolling to 0.8 mm in sheet thickness and was subjected to cold-rolled sheet annealing under the conditions shown in Table 2 to obtain a cold-rolled and annealed sheet. Except to No. 13 and No. 16, the atmosphere gas in all heating and cooling processes in the temperature range of 200° C. or more during the annealing was the same atmosphere gas as in the nitrogen-enriched layer formation treatment presented in Table 2. In No. 13 and No. 16, the atmosphere gas in the heating process of 200° C. to 800° C. during the annealing was a 100% H<sub>2</sub> gas atmosphere, and the atmosphere gas in the heating process in the other temperature range and the cooling process to 200° C. was the same atmosphere gas as in the nitrogen-enriched layer forming treatment presented in Table 2.

Note that in a situation in which the external appearance of the sheet was deep yellow or blue, it was judged that a thick oxide film had been formed and +20 A/dm<sup>2</sup> → -20 A/dm<sup>2</sup> electrolytic picking was performed twice, with different electrolysis times, in a mixed acid solution of 150 g/l of nitric acid and 5 g/l of hydrochloric acid at a temperature of 55° C.

Evaluation of (1) ductility and measurement of (2) nitrogen concentration at nitrogen-enriched layer were performed as described below for each cold-rolled and annealed sheet obtained as described above.

Furthermore, brazing was carried out for each cold-rolled and annealed sheet using a Ni-containing brazing metal and the cold-rolled and annealed sheet was evaluated after brazing in terms of (3) corrosion resistance and (4) brazing properties. The evaluation of (4) brazing properties was performed as described below for (a) joint gap infiltration of the brazing metal and (b) joint strength of a brazed part.

### (1) Ductility Evaluation

A JIS No. 13B tensile test piece was sampled at a right angle to the rolling direction from each of the cold-rolled and annealed sheets described above, a tensile test was carried out in accordance with JIS Z 2241, and ductility was evaluated using the following standard. The evaluation results are shown in Table 2.

Good (pass): Elongation after fracture was 20% or greater  
Poor (fail): Elongation after fracture was less than 20%  
(2) Measurement of Nitrogen Concentration at Nitrogen-Enriched Layer

The surface of each of the cold-rolled and annealed sheets was analyzed by glow discharge optical emission spectroscopy (hereinafter referred to as GDS). First, samples with

different sputtering times from the surface layer were prepared and cross-sections thereof were observed by SEM in order to prepare a calibration curve for a relationship between sputtering time and depth.

Nitrogen concentration was measured while performing sputtering from the surface of the steel to a depth of 0.50  $\mu\text{m}$ . Herein, the measured values of Cr and Fe are fixed at the depth of 0.50  $\mu\text{m}$  and thus a measured value for nitrogen concentration at the depth of 0.50  $\mu\text{m}$  was taken to be the nitrogen concentration of the base material (steel substrate).

A highest peak value (maximum value) among measured nitrogen concentration values within 0.05  $\mu\text{m}$  of the steel surface was divided by the measured nitrogen concentration value at the depth of 0.50  $\mu\text{m}$  and the resultant value was multiplied by a nitrogen concentration of the steel obtained by chemical analysis to give a value that was taken to be a nitrogen concentration peak value at a depth of within 0.05  $\mu\text{m}$  of the surface. Nitrogen concentration peak values that were obtained are shown in Table 2.

### (3) Evaluation of Corrosion Resistance

After brazing was carried out for each of the cold-rolled and annealed sheets, a 20 mm square test piece was sampled from a part to which brazing metal was not attached, and the test piece was covered by a sealing material, but leaving a 11 mm square measurement surface. Thereafter, the test piece was immersed in a 3.5% NaCl solution at 30° C. and a corrosion resistance test was conducted in accordance with JIS G 0577 with the exception of the NaCl concentration. Pitting corrosion potentials  $V_{c100}$  were measured and evaluated using the following standard. The evaluation results are shown in Table 2.

Good: the pitting potential  $V_{c100}$  was 100 (mV vs SCE) or more.

Poor: the pitting potential  $V_{c100}$  was less than 100 (mV vs SCE).

### (4) Evaluation of Brazing Properties

#### (a) Infiltration of Brazing Metal into Joint Gap

As illustrated in FIG. 1, a 30 mm square sheet and a 25 mm×30 mm sheet were cut out from each of the cold-rolled and annealed sheets and these two sheets were overlapped and clamped in place using a clamp jig with a fixed torque force (170 kgf). Next, 1.2 g of a brazing metal was applied onto an end surface of one of the sheets and brazing was carried out. After the brazing, the degree to which the brazing metal had infiltrated between the sheets was visually confirmed from a side surface part of the overlapped sheets and was evaluated using the following standard. The evaluation results are shown in Table 2. Note that in the drawings,

the reference sign 1 indicates the cold-rolled and annealed sheet and the reference sign 2 indicates the brazing metal.

Excellent (pass, particularly good): Brazing metal infiltration to opposite end relative to application end

Satisfactory (pass): Brazing metal infiltration over at least 50% and less than 100% of the overlapping length of the two sheets

Unsatisfactory (fail): Brazing metal infiltration over at least 10% and less than 50% of the overlapping length of the two sheets

10 Poor (fail): Brazing metal infiltration over less than 10% of the overlapping length of the two sheets

#### (b) Joint strength of brazed part

As illustrated in FIG. 2, portions of a JIS No. 13B tensile test piece that had been split at the center thereof were overlapped by 5 mm and were clamped in place using a clamp jig. Next, brazing was carried out by applying 0.1 g of a brazing metal to an overlapping part of one of the portions. After the brazing, a tensile test was conducted at normal temperature and joint strength of the brazed part was evaluated using the following standard. The evaluation results are shown in Table 2. Note that in the drawings, reference sign 3 indicates the tensile test piece.

Excellent (pass, particularly good): No brazed part fracture even at 95% or greater of tensile strength of base material (base material part fracture)

Satisfactory (pass): Brazed part fracture at 95% or greater of tensile strength of base material

Unsatisfactory (fail): Brazed part fracture at 50% or greater and less than 95% of tensile strength of base material

30 Poor (fail): Brazed part fracture at less than 50% of tensile strength of base material

In each evaluation of brazing properties described above, the brazing metal was a typical Ni-containing brazing metal BNi-5 (19% Cr and 10% Si in a Ni matrix) stipulated by Japanese Industrial Standards. The brazing was carried out in a sealed furnace. Furthermore, brazing was carried out in a high vacuum atmosphere of  $10^{-2}$  Pa and was also carried out in an Ar carrier gas atmosphere by enclosing Ar with a pressure of 100 Pa after forming a high vacuum. A temperature pattern of the heat treatment involved performing treatment with a heating rate of 10° C./s, a first soaking time (step of equilibrating overall temperature) of 1800 s at 1060° C., a heating rate of 10° C./s, and a second soaking time (step of actually carrying out brazing at a temperature equal to or higher than the melting point of the brazing metal) of 600 s at 1170° C., followed by furnace cooling and purging of the furnace with external air (atmosphere) once the temperature had fallen to 200° C.

TABLE 1

| Steel | Chemical composition (mass %) |      |      |       |       |      |      |      |      |       |      |      |      |      |        | Remarks |                  |
|-------|-------------------------------|------|------|-------|-------|------|------|------|------|-------|------|------|------|------|--------|---------|------------------|
|       | ID                            | C    | Si   | Mn    | P     | S    | Cr   | Cu   | Ni   | Nb    | N    | Mo   | Al   | Ti   | V      | Ca      |                  |
| AA    | 0.005                         | 0.25 | 0.21 | 0.026 | 0.001 | 18.9 | 0.45 | 0.21 | 0.45 | 0.007 | —    | —    | —    | —    | —      | —       | Conforming steel |
| AB    | 0.004                         | 0.31 | 0.21 | 0.023 | 0.001 | 22.8 | 0.38 | 0.19 | 0.33 | 0.008 | —    | —    | —    | —    | —      | —       | Conforming steel |
| AC    | 0.004                         | 0.26 | 0.18 | 0.024 | 0.001 | 19.5 | 0.26 | 0.32 | 0.36 | 0.008 | —    | —    | —    | —    | —      | —       | Conforming steel |
| AD    | 0.006                         | 0.28 | 0.21 | 0.023 | 0.001 | 19.2 | 0.42 | 0.19 | 0.34 | 0.009 | 0.15 | —    | 0.11 | —    | —      | 0.0004  | Conforming steel |
| AE    | 0.007                         | 0.21 | 0.22 | 0.027 | 0.001 | 22.5 | 0.68 | 0.28 | 0.20 | 0.009 | —    | —    | 0.15 | —    | 0.0015 | —       | Conforming steel |
| AF    | 0.010                         | 0.13 | 0.11 | 0.025 | 0.002 | 19.0 | 0.38 | 0.21 | 0.49 | 0.011 | —    | —    | —    | 0.12 | —      | 0.0006  | Conforming steel |
| AG    | 0.006                         | 0.15 | 0.13 | 0.023 | 0.001 | 22.7 | 0.20 | 0.38 | 0.36 | 0.006 | —    | 0.09 | —    | 0.08 | —      | —       | Conforming steel |

TABLE 1-continued

| Steel | Chemical composition (mass %) |      |      |       |       |      |      |      |      |       |      |      |    |    |   |    |                   |
|-------|-------------------------------|------|------|-------|-------|------|------|------|------|-------|------|------|----|----|---|----|-------------------|
|       | ID                            | C    | Si   | Mn    | P     | S    | Cr   | Cu   | Ni   | Nb    | N    | Mo   | Al | Ti | V | Ca | B                 |
| AH    | 0.006                         | 0.22 | 0.35 | 0.025 | 0.002 | 17.5 | 0.44 | 0.29 | 0.43 | 0.007 | 0.18 | 0.05 | —  | —  | — | —  | Conforming steel  |
| BA    | 0.007                         | 0.15 | 0.23 | 0.022 | 0.001 | 15.5 | 0.21 | 0.25 | 0.33 | 0.006 | —    | —    | —  | —  | — | —  | Comparative steel |
| BB    | 0.005                         | 0.22 | 0.12 | 0.023 | 0.002 | 18.6 | 0.16 | 0.18 | 0.34 | 0.008 | —    | —    | —  | —  | — | —  | Comparative steel |
| BC    | 0.006                         | 0.18 | 0.22 | 0.020 | 0.001 | 19.3 | 0.28 | 0.21 | 0.16 | 0.008 | —    | —    | —  | —  | — | —  | Comparative steel |

TABLE 2

| Steel<br>No. | Steel<br>ID | Annealing conditions                                       |                                                             |                           |                     |                                                                             |    | Time of nitrogen-<br>enriched layer<br>pickling |  |
|--------------|-------------|------------------------------------------------------------|-------------------------------------------------------------|---------------------------|---------------------|-----------------------------------------------------------------------------|----|-------------------------------------------------|--|
|              |             | Dew point in<br>temperature range<br>of 600° C. to 800° C. | Atmosphere of nitrogen-<br>enriched layer forming treatment |                           |                     | Temperature of<br>nitrogen-enriched<br>layer forming<br>treatment<br>(° C.) |    |                                                 |  |
|              |             |                                                            | H <sub>2</sub><br>(vol %)                                   | N <sub>2</sub><br>(vol %) | Dew point<br>(° C.) |                                                                             |    |                                                 |  |
| 1            | AA          | -35                                                        | 75                                                          | 25                        | -35                 | 960                                                                         | 30 | Not performed                                   |  |
| 2            | AA          | -40                                                        | 70                                                          | 30                        | -40                 | 960                                                                         | 30 | Not performed                                   |  |
| 3            | AA          | -45                                                        | 5                                                           | 95                        | -45                 | 970                                                                         | 60 | Performed                                       |  |
| 4            | AB          | -35                                                        | 50                                                          | 50                        | -25                 | 950                                                                         | 30 | Not performed                                   |  |
| 5            | AB          | -45                                                        | 75                                                          | 25                        | -45                 | 960                                                                         | 30 | Not performed                                   |  |
| 6            | AB          | -36                                                        | 10                                                          | 90                        | -25                 | 960                                                                         | 40 | Performed                                       |  |
| 7            | AC          | -25                                                        | 75                                                          | 25                        | -20                 | 960                                                                         | 40 | Not performed                                   |  |
| 8            | AC          | -39                                                        | 85                                                          | 15                        | -45                 | 970                                                                         | 30 | Not performed                                   |  |
| 9            | AD          | -41                                                        | 75                                                          | 25                        | -35                 | 960                                                                         | 30 | Not performed                                   |  |
| 10           | AD          | -45                                                        | 75                                                          | 25                        | -55                 | 960                                                                         | 30 | Not performed                                   |  |
| 11           | AE          | -40                                                        | 90                                                          | 10                        | -45                 | 960                                                                         | 30 | Not performed                                   |  |
| 12           | AE          | -32                                                        | 10                                                          | 90                        | -20                 | 960                                                                         | 30 | Performed                                       |  |
| 13           | AF          | -35                                                        | 90                                                          | 10                        | -25                 | 960                                                                         | 30 | Not performed                                   |  |
| 14           | AF          | -44                                                        | 75                                                          | 25                        | -45                 | 930                                                                         | 30 | Not performed                                   |  |
| 15           | AG          | -47                                                        | 75                                                          | 25                        | -45                 | 930                                                                         | 30 | Not performed                                   |  |
| 16           | AH          | -46                                                        | 75                                                          | 25                        | -45                 | 930                                                                         | 30 | Not performed                                   |  |
| 17           | AA          | <u>-15</u>                                                 | 75                                                          | 25                        | <u>-10</u>          | 960                                                                         | 30 | Not performed                                   |  |
| 18           | AB          | -26                                                        | 100                                                         | 0                         | -25                 | 970                                                                         | 30 | Not performed                                   |  |
| 19           | AC          | -40                                                        | 75                                                          | 25                        | -45                 | <u>860</u>                                                                  | 30 | Not performed                                   |  |
| 20           | <u>BA</u>   | -40                                                        | 75                                                          | 25                        | -45                 | 960                                                                         | 30 | Not performed                                   |  |
| 21           | <u>BB</u>   | -25                                                        | 5                                                           | 95                        | -30                 | 920                                                                         | 30 | Performed                                       |  |
| 22           | <u>BC</u>   | -26                                                        | 75                                                          | 25                        | -25                 | 960                                                                         | 30 | Not performed                                   |  |
| 23           | AB          | <u>-15</u>                                                 | 75                                                          | 25                        | -25                 | 950                                                                         | 30 | Not performed                                   |  |

TABLE 2-continued

| No. | Ductility evaluation | enriched layer (mass %) | Corrosion resistance evaluation | Brazing properties evaluation (brazing in high vacuum) |                            | Brazing properties evaluation (brazing in Ar atmosphere) |                            | Remarks             |
|-----|----------------------|-------------------------|---------------------------------|--------------------------------------------------------|----------------------------|----------------------------------------------------------|----------------------------|---------------------|
|     |                      |                         |                                 | Nitrogen concentration peak value of nitrogen-         | Brazing metal infiltration | Brazed part joint strength                               | Brazing metal infiltration |                     |
|     |                      |                         |                                 |                                                        |                            |                                                          |                            |                     |
| 1   | Good                 | 0.22                    | Good                            | Excellent                                              | Excellent                  | Excellent                                                | Excellent                  | Example             |
| 2   | Good                 | 0.19                    | Good                            | Excellent                                              | Excellent                  | Excellent                                                | Satisfactory               | Example             |
| 3   | Good                 | 0.08                    | Good                            | Satisfactory                                           | Satisfactory               | Satisfactory                                             | Satisfactory               | Example             |
| 4   | Good                 | 0.28                    | Good                            | Excellent                                              | Excellent                  | Excellent                                                | Satisfactory               | Example             |
| 5   | Good                 | 0.21                    | Good                            | Excellent                                              | Excellent                  | Excellent                                                | Excellent                  | Example             |
| 6   | Good                 | 0.06                    | Good                            | Satisfactory                                           | Satisfactory               | Satisfactory                                             | Satisfactory               | Example             |
| 7   | Good                 | 0.08                    | Good                            | Satisfactory                                           | Satisfactory               | Satisfactory                                             | Satisfactory               | Example             |
| 8   | Good                 | 0.18                    | Good                            | Excellent                                              | Satisfactory               | Excellent                                                | Satisfactory               | Example             |
| 9   | Good                 | 0.20                    | Good                            | Satisfactory                                           | Satisfactory               | Satisfactory                                             | Satisfactory               | Example             |
| 10  | Good                 | 0.29                    | Good                            | Satisfactory                                           | Satisfactory               | Satisfactory                                             | Satisfactory               | Example             |
| 11  | Good                 | 0.08                    | Good                            | Satisfactory                                           | Satisfactory               | Satisfactory                                             | Satisfactory               | Example             |
| 12  | Good                 | 0.12                    | Good                            | Satisfactory                                           | Satisfactory               | Satisfactory                                             | Satisfactory               | Example             |
| 13  | Good                 | 0.21                    | Good                            | Excellent                                              | Excellent                  | Excellent                                                | Excellent                  | Example             |
| 14  | Good                 | 0.18                    | Good                            | Excellent                                              | Excellent                  | Excellent                                                | Excellent                  | Example             |
| 15  | Good                 | 0.27                    | Good                            | Satisfactory                                           | Satisfactory               | Satisfactory                                             | Satisfactory               | Example             |
| 16  | Good                 | 0.29                    | Good                            | Excellent                                              | Excellent                  | Excellent                                                | Excellent                  | Example             |
| 17  | Good                 | 0.02                    | Good                            | Unsatisfactory                                         | Poor                       | Unsatisfactory                                           | Poor                       | Comparative Example |
| 18  | Good                 | 0.01                    | Good                            | Unsatisfactory                                         | Poor                       | Unsatisfactory                                           | Poor                       | Comparative Example |
| 19  | Poor                 | 0.01                    | Good                            | Unsatisfactory                                         | Poor                       | Unsatisfactory                                           | Poor                       | Comparative Example |
| 20  | Good                 | 0.18                    | Poor                            | Excellent                                              | Satisfactory               | Satisfactory                                             | Satisfactory               | Comparative Example |
| 21  | Good                 | 0.09                    | Poor                            | Satisfactory                                           | Satisfactory               | Satisfactory                                             | Satisfactory               | Comparative Example |
| 22  | Good                 | 0.12                    | Poor                            | Excellent                                              | Satisfactory               | Satisfactory                                             | Satisfactory               | Comparative Example |
| 23  | Good                 | 0.02                    | Good                            | Unsatisfactory                                         | Poor                       | Unsatisfactory                                           | Poor                       | Comparative Example |

Table 2 shows that for each of Examples 1-16, infiltration of the brazing metal into the joint gap was good and joint strength of the brazed part was good. Accordingly, it was demonstrated that these examples display good brazing properties even when a Ni-containing brazing metal is used. Furthermore, these examples had good corrosion resistance and ductility.

In contrast, good brazing properties or good corrosion resistance were not obtained in Comparative Examples 17-23 for which the chemical composition or the nitrogen concentration peak value was outside of the appropriate range.

## INDUSTRIAL APPLICABILITY

The present disclosure enables a ferritic stainless steel to be obtained that can be suitably used for heat exchanger components and the like of exhaust heat recovery units and EGR coolers that are assembled by brazing, and is therefore extremely useful in industry.

## REFERENCE SIGNS LIST

1 cold-rolled and annealed sheet

2 brazing metal

3 tensile test piece

The invention claimed is:

1. A ferritic stainless steel comprising a chemical composition consisting of, in mass %: 0.003% to 0.025% of C; 0.05% to 1.00% of Mn;

0.04% or less of P;

0.01% or less of S;

16.0% to 23.0% of Cr;

0.20% to 0.80% of Cu;

0.05% to 0.60% of Ni;

0.20% to 0.70% of Nb;

0.005% to 0.020% of N; and

the balance being Fe and incidental impurities, wherein a nitrogen-enriched layer is present that has a nitrogen concentration peak value of 0.03 mass % to 0.30 mass % at a depth of within 0.05  $\mu\text{m}$  of a surface of the steel.

0.05% to 1.00% of Mn;

0.04% or less of P;

0.01% or less of S;

16.0% to 23.0% of Cr;

0.20% to 0.80% of Cu;

0.05% to 0.60% of Ni;

0.20% to 0.70% of Nb;

0.005% to 0.020% of N; and

the balance being Fe and incidental impurities, wherein a nitrogen-enriched layer is present that has a nitrogen concentration peak value of 0.03 mass % to 0.30 mass % at a depth of within 0.05  $\mu\text{m}$  of a surface of the steel.

2. A ferritic stainless steel comprising a chemical composition consisting of, in mass %:

0.003% to 0.025% of C;

0.05% to 1.00% of Si;

0.05% to 1.00% of Mn;

0.04% or less of P;

0.01% or less of S;

16.0% to 23.0% of Cr;

0.20% to 0.80% of Cu;

0.05% to 0.60% of Ni;

0.20% to 0.70% of Nb;

0.005% to 0.020% of N; and

one or more of:

0.05% to 0.20% of Mo;

0.01% to 0.15% of Al;

0.01% to 0.15% of Ti;

0.01% to 0.20% of V;

**17**

0.0003% to 0.0030% of Ca; and  
0.0003% to 0.0030% of B,

the balance being Fe and incidental impurities, wherein a nitrogen-enriched layer is present that has a nitrogen concentration peak value of 0.03 mass % to 0.30 mass % at a depth of within 0.05  $\mu\text{m}$  of a surface of the steel.

**3.** A process for producing the ferritic stainless steel of claim 1, the process comprising:

hot rolling a slab having the chemical composition of claim 1 to form a hot-rolled sheet;

optionally performing hot-rolled sheet annealing on the hot-rolled sheet; and

performing a combination of cold rolling and annealing on the hot-rolled sheet one or more times,

wherein a cold-rolled sheet after subjection to final cold rolling is heated in final annealing with a dew point of an atmosphere in a temperature range of 600° C. to 800° C. being 20° C. or lower, and subjected to a nitrogen-enriched layer forming treatment at a tem-

10

15

**18**

perature of 900° C. or higher in an atmosphere of 20° C. or lower in dew point and 5 vol % or more in nitrogen concentration.

**4.** A process for producing the ferritic stainless steel of claim 2, the process comprising:

hot rolling a slab having the chemical composition of claim 2 to form a hot-rolled sheet;

optionally performing hot-rolled sheet annealing on the hot-rolled sheet; and

performing a combination of cold rolling and annealing on the hot-rolled sheet one or more times,

wherein a cold-rolled sheet after subjection to final cold rolling is heated in final annealing with a dew point of an atmosphere in a temperature range of 600° C. to 800° C. being -20° C. or lower, and subjected to a nitrogen-enriched layer forming treatment at a temperature of 900° C. or higher in an atmosphere of -20° C. or lower in dew point and 5 vol % or more in nitrogen concentration.

\* \* \* \* \*